

## UNITED STATES PATENT OFFICE.

JAMES W. WEIR, OF FILLMORE, CALIFORNIA.

## PROCESS FOR REFINING MINERAL LUBRICATING OILS.

No Drawing.

Application filed May 14, 1925. Serial No. 30,355.

This invention relates to the manufacture of lubricating oils, and refers particularly to improvements in the treatment of lubricating oil stocks from mineral or petroleum oils with sulfuric acid.

In the treatment and refining of lubricating oil stocks with mineral petroleum oils, the stock is commonly treated with sulfuric acid. The sulfuric acid is added to the lubricating oil stock and the admixture agitated for a period of time until the purification reaction substantially ceases. As a result of such reaction, a quantity of sludge or partially spent acid is formed. The strength of sulfuric acid in the produced sludge, while at too low a potential strength for further refining of the lubricating oil stock commingled therewith, still possesses considerable potential strength in reference to its ability to treat untreated lubricating stock, or certain treated or untreated stocks of different grade.

In an ordinary process of refining, however, this residual sulfuric acid strength of the sludge is not utilized. Moreover, in the practical application of acid in the treatment of lubricating oil stocks, it is difficult to apply the acid to the stock so as to secure a substantially and economical efficiency in the reaction between the lubricating oil stock and acid without at the same time causing a violent reaction to take place. The effect of a too vigorous reaction between sulfuric acid and certain oil stocks imparts to the stock a bluish fluorescence or bloom, whereas otherwise the lubricating oil stock would possess an olive green bloom or fluorescence by reflected light. Lubricating oil with a bluish fluorescence or bloom is generally considered of low grade in the market.

It is an object of the present invention to provide a method of treating lubricating oil stocks by which the sulfuric acid employed is more efficiently utilized and by which a modified action of sulfuric acid upon lubricating oil stocks is obtained, so that this formation or imparting of a bluish fluorescence or bloom to the finished stock is avoided and a superior lubricating oil stock thus provided at a lower rate of acid consumption.

The process is particularly adapted to the treatment of lubricating oils wherein

it is desired to produce a lubricating oil of intermediate viscosity or color from a stock of low viscosity and light color and a stock of relatively high viscosity and dark color.

It has hitherto been particularly difficult to treat, for example, heavy steam refined stock to a relatively light color as compared to the original stocks. Attempts to refine, treat and filter to such a comparatively light color, generally result in the imparting to such stock of an undesirable bluish fluorescence or bloom as viewed by reflected light. It is a common practice to process these heavy viscous stocks as far as possible, and rely upon the treatment of the lighter stocks with which they are finally to be blended as a merchantable product to bring the blended finished oil up to the desired standard of color.

By the method of this invention, these heavy viscous stocks may be treated with more efficiency and with less tendency to produce a stock of the undesired or bluish fluorescence. The method effects a modified sulfuric acid treatment secured by mixing such heavy stocks with an admixture of lighter, less viscous stocks and sulfuric acid sludge resulting from the treatment of such light stock with sulfuric acid. The mass is then agitated together so that the acid sludge will effect a purification of the heavy viscous stock under conditions which are found to substantially retard the imparting of a bluish fluorescence or bloom to the resultant product. This is due to the presence of the less viscous stock and the fact that the potential sulfuric acid strength of the sludge is materially reduced.

The invention is particularly useful in connection with the production of blended intermediate stock from the use of a light and heavy oil stock. The method of treatment or modified sulfuric acid treatment, however, may be utilized wherever, following a sulfuric acid treatment of one lubricating oil stock and prior to the removal of the sludge formed thereby, any other additional lubricating oil stock is added thereto and the mass agitated together for the refining of said additional stock. In any case, the resultant action upon the second stock is obtained, through a treatment thereof by a hitherto waste material, the purification being accomplished without effecting

the vigorous reaction which causes the impartation of a bluish fluorescence or bloom to the oil.

The objects and advantages of the process 5 will be more fully understood from a detailed description of a preferred example or illustration of a process embodying the invention.

Lubricating oil stock of relatively low 10 viscosity is commingled with approximately fifteen pounds of sulfuric acid per barrel of stock under treatment and maintained in intimate contact for approximately forty-five minutes. The stock is then allowed to 15 settle, after which the sludge resulting from this acid treatment is preferably withdrawn. Then approximately twenty pounds of sulfuric acid per barrel of stock is added and similarly commingled and maintained in 20 intimate contact with the oil stock for approximately forty-five minutes. Then while the oil and admixed acid are still being commingled and maintained in intimate contact, filtered cylinder stock or lubricating oil stock 25 of relatively high viscosity is added and commingled with the first stock and sludge therefrom while still remaining therein for a period of approximately forty-five minutes. For example, 20% by volume of the 30 second stock may be added. In this way, the sludge produced from the second sulfuric acid treatment of the first or lighter oil stock is caused to purify the second or added heavier oil stock, the purification thus 35 being effected by a comparatively valueless material, and the sulfuric acid employed being more efficiently utilized. Moreover, the resulting action is found to be substantially less vigorous and proceeds without the im- 40 parting of a bluish fluorescence or bloom to the blended finished stock.

Subsequent to such treatment, the sludge is permitted to settle from the oil stock and is then withdrawn.

45 After such an acid treatment, the lubricating oil stock may be finished by any preferred method, such for example, as washing or gathering by water and neutralization with an alkali soda, but preferably is 50 finished in the following manner:

There still remains suspended in the oil a certain percentage of finely divided sludge 55 or "pepper" which will not settle out of the lubricating oil stock and should be removed to obtain a lubricating oil of high purity. This "pepper" may be removed by gathering the same with a comminuted solid adsorbent material, the same being agitated with the stock at a temperature below the decom- 60 posing temperature of the sludge present. The comminuted solid adsorbent material may be added at the rate of one ton of the solid substance to thirty thousand gallons of the oil stock. Comminuted granite, di- 65 atomaceous earth, decolorizing clays or ful-

ler's earth are examples of solid materials which may be employed. The comminuted substance, with the sludge gathered and adhering thereto, is then separated from the oil stock.

The oil stock still contains a quantity of acid reaction products or acid sludge in colloidal suspension or otherwise remaining in the oil stock, and to remove such material, a comminuted solid adsorbent material is 70 added to the oil at the rate of approximately one ton of the said solid to 5,000 gallons of the oil stock. The comminuted solid may be the same or different than that employed in the previous step. The admixture is then 75 agitated and heated to a temperature sufficient to cause the sludge present to decompose and liberate carbon dioxide. The decomposing sludge will adhere to the comminuted substance commingled with the oil 80 and can then be removed.

The temperature of the treatment is 180° F. or above and may be as high as any temperature below the vaporizing temperature of the oil stock, although relatively 85 lower temperatures, such as 300° F. are preferred. During the agitation of the oil and solids together, an inert gas may be blown through the same to assist in the removal of the sulfur dioxide. Subsequent to such 90 treatment, the lubricating oil stock is separated from the remainder of the mass and then, if necessary, is brightened by blowing with air in the usual manner.

This method of removing acid reaction 100 products from the oil by adsorption with a comminuted solid substance is accompanied by no chemical reaction, and therefore no injurious compounds are formed which remain in the oil or require removal by fur- 105 ther process.

While I have described in detail the preferred method of refining lubricating oils, it is understood that various modifications 110 may be made in the details of the method and process, without departing from the spirit of the invention, and the invention is therefore not limited to the specific details set forth for the purpose of illustration, but includes all such modifications and substi- 115 tutions as come within the scope of the appended claims.

I claim:—

1. The process of refining lubricating oil stocks, which comprises treating relatively 120 low viscosity lubricating oil stock with sulfuric acid until the action of the acid upon said stock is substantially complete, then without removing the produced sludge from said treatment introducing relatively high viscosity lubricating oil stock to the admixture and commingling the same therewith, whereby the added oil stock is reacted upon by the acid sludge resulting from the sulfuric acid treatment of the original stock. 125

2. In a process of refining lubricating oil stocks, the method which comprises treating a relatively low viscosity lubricating oil stock with sulfuric acid until the resultant reaction is substantially complete, then without removing the produced sludge from said treatment adding a relatively high viscosity lubricating oil stock to the admixture, continuing the treatment to thus effect a modified reaction upon the added heavy stock, and separating the blended lubricating oil stock from the resultant sludge.
3. The method of refining a lubricating oil stock, which comprises treating relatively low viscosity lubricating oil stock with sulfuric acid and then, without removing the produced sludge from such treatment, adding a second relatively high viscosity lubricating oil stock to the admixture and continuing the treatment, settling and removing the major portion of the sludge, and then gathering and removing a further quantity of the sludge remaining in the oil stock by treatment with comminuted solid adsorbent material.
4. The method of refining a lubricating oil stock, which comprises treating a lubricating oil of relatively low viscosity with sulfuric acid, then without removing the sludge, adding a lubricating oil of relatively higher viscosity, settling and removing the major portion of the sludge, and gathering and removing a further quantity of the remainder of the sludge by the treatment with comminuted solid adsorbent material.
5. The method of refining lubricating oil stock, which comprises treating a lubricating oil of relatively low viscosity with sulfuric acid, then without removing the sludge adding a lubricating oil of relatively higher viscosity and continuing the treatment, sepa-
- rating the major portion of the sludge therefrom, commingling the lubricating oil stock with a comminuted solid adsorbent material at a temperature sufficient to decompose the sludge present, and separating the adsorbent material with the material adsorbed from the oil stock.
6. The method of refining lubricating oil stocks, which comprises treating a lubricating oil of relatively low viscosity with sulfuric acid, then without removing the sludge produced, adding a lubricating oil of relatively higher viscosity and continuing the treatment, removing the major portion of the sludge therefrom, and gathering the suspended sludge from the lubricating oil stock by adding and commingling therewith a comminuted solid adsorbent material at a temperature below the decomposing temperature of the sludge.
7. The method of refining lubricating oil stocks, which comprises treating a lubricating oil of relatively low viscosity with sulfuric acid, then without removing the sludge, adding a lubricating oil of relatively higher viscosity and continuing the treatment, removing the major portion of the sludge formed, gathering the suspended sludge by adding and commingling therewith a solid adsorbent material at a temperature below the decomposing temperature of the sludge, removing the adsorbent material and gathered sludge, agitating the oil stock with comminuted solid adsorbent material at a temperature sufficient to decompose the remaining sludge and liberate sulfur dioxide, and then separating the oil stock from the mass.

Signed at Los Angeles, Calif., this 4 day of May 1925.

JAMES W. WEIR.